

OF INVENTION AND OF THIS INVENTION. THE  
BE SUBJECTIVE AND NOT THE INVENTION. THE  
INVENTION IS NOT SUBJECTIVE AND NOT THE  
INVENTION.

2,990,346

## IRRADIATION OF SODIUM BASE GREASES

Alvin M. Natkin, Metuchen, John J. Kolfenbach, North Plainfield, and Eric O. Forster, Scotch Plains, N. J., assignors to Esso Research and Engineering Company, a corporation of Delaware

No Drawing. Filed Mar. 23, 1956, Ser. No. 573,324

3 Claims. (Cl. 204—154)

This invention relates to lubricating grease compositions, and more particularly to a process of improving certain physical properties of sodium base lubricating greases. In brief compass, the invention pertains to subjecting sodium base lubricating greases to high intensity ionizing radiation to obtain greases having color and odor improvement as well as other desirable grease characteristics.

In the prior art, improved physical properties of lubricating greases have usually been attained through the use of special refining or finishing methods, unique thickening agents or oil bases and particular additives. In accordance with the present invention, it has now been found that physical properties of sodium base lubricating greases can be markedly improved by irradiation of the greases with high intensity ionizing radiation comprising gamma rays. This process has the advantages that usually it is less expensive than the prior art methods, it is more easily controlled, and it is more readily adapted to a continuous operation.

The gamma rays with which the lubricating greases of the invention are irradiated may be derived from the radioactive decay of certain natural or artificially radioactive elements or isotopes such as radium 226, radium A, radium B, radium C, radium D, thallium 210, cobalt 60, cesium 137, europium 152-154, cesium 134, cerium 144, silver 110, thulium 170, tantalum 182, scandium 46, terbium 160 or iridium 192 or from chemical compounds of or materials containing such elements or isotopes. The gamma rays may also be derived from suitably shielded radiation produced in nuclear reactors, i.e. atomic piles, or from the spent fuel elements obtained from the operation of such reactors.

In general, undisturbed gamma ray fluxes within the range of about  $10^3$  to  $6 \times 10^8$ , usually about  $10^4$  to  $3 \times 10^8$ , roentgens per hour, such as that derived from a cobalt 60 source, will be employed in irradiating the sodium base lubricating greases. The time of irradiation will depend upon the degree of change in the physical properties of the lubricating greases desired as well as upon the radiation dosage rate. The total radiation dosage (based on undisturbed radiation field conditions, i.e. conditions prior to the introduction of the lubricating oil into the radiation field) will ordinarily be within the range of about  $10^5$  to  $3 \times 10^{10}$ , preferably about  $10^6$  to  $3 \times 10^9$ , roentgens of gamma rays. Thus, irradiation time may vary from about 0.01 to 3000 hours, preferably about 0.5 to 200 hours. For the purposes of this invention, however, the lubricating grease need only be irradiated for a sufficient period of time to obtain the desired change in physical properties.

The sodium base greases may also be irradiated in an atomic pile wherein the radiation will consist primarily of fast and slow neutrons and gamma rays.

The lubricating greases employed in the invention may be any of the sodium soap thickened greases described in chapter 11 of Boner's "Manufacture and Application of Lubricating Greases" (Reinhold Publishing Corp.). The naturally occurring or synthetic fats or fatty acids employed in formulating the sodium grease-thickening soaps may be selected from the commonly known grease-making materials. Examples of these materials include saturated or unsaturated fatty acids having iodine num-

bers within the range of about 0 to 154 and having about 12 to 30, preferably about 18 to 22, carbon atoms per molecule, such as lauric, myristic, palmitic, stearic, 12-hydroxy stearic, 9,10-dihydroxy stearic, behenic, myristoleic, palmitoleic, oleic, linoleic, lignoceric, ricinoleic and erucic acids, cottonseed oil fatty acids, animal fatty acids, palm oil fatty acids, hydrogenated fish oil fatty acids and their mixtures and/or their glycerides such as lard, beef, rapeseed, palm, menhaden, herring, castor oils, etc.

The lubricating oil menstruum may be any of the conventionally used mineral, animal, vegetable or synthetic lubricating oils. In general, these lubricating oils should have a viscosity of about 50 to 2000 SUS at 100° F. and about 35 to 200 SUS at 210° F., an A.S.T.M. pour point of about +20 to -75° F., a flash point of about 350° to 650° F. and a viscosity index of about 0 to 60 or higher. Conventionally refined and treated mineral oil base stocks which are derived from paraffinic, naphthenic and mixed base crudes and have the properties listed above are especially useful in preparing the sodium base lubricating grease compositions.

The synthetic lubricating oils which may also be employed include esters of monobasic acids (e.g. an ester of C<sub>8</sub> Oxo alcohol with C<sub>8</sub> Oxo acid, an ester of C<sub>13</sub> Oxo alcohol with octanoic acid, etc.), esters of dibasic acids (e.g. di-2-ethyl hexyl sebacate, di-nonyl adipate, etc.), esters of glycols (e.g. C<sub>13</sub> Oxo acid diester of tetraethylene glycol, etc.), complex esters (e.g. the complex ester formed by reacting one mol of tetraethylene glycol with two moles of sebacic acid and two moles of 2-ethylhexanol, or the complex ester formed by reacting one mol of tetraethylene glycol, one mol of adipic acid, one mol of C<sub>8</sub> Oxo alcohol and one mol of C<sub>8</sub> Oxo acid, etc.), esters of phosphoric acid (e.g. the ester formed by contacting three moles of the mono-methyl ether of ethylene glycol with one mol of phosphorous oxychloride, etc.), halocarbon oils (e.g. the polymer of chlorotrifluoroethylene containing twelve recurring units of chlorotrifluoroethylene), carbonates (e.g. the carbonate formed by reacting C<sub>8</sub> Oxo alcohol with ethyl carbonate to form a half ester and reacting this half ester with tetraethylene glycol), mercaptals (e.g. the mercaptal formed by reacting 2-ethyl hexyl mercaptan with formaldehyde), formals (e.g. the formal formed by reacting C<sub>13</sub> Oxo alcohol with formaldehyde), polyglycol type synthetic oils (e.g. the compounds formed by condensing butyl alcohol with fourteen units of propylene oxide, etc.), or mixtures of the above in any proportions.

The preparation of the sodium soap thickened greases may be carried out by any of the conventional processes described in sections 11:4 to 11:13 of chapter 11 of Boner, supra. Since the preparation of lubricating greases is not directly related to the present invention, these methods need not be described in detail.

In accordance with one aspect of this invention, a sodium base grease wherein the thickener is prepared from certain glyceride-type fats and oils may be advantageously subjected to high intensity ionizing radiation comprising gamma rays. The saponifiable material used in preparing these greases may be saturated, unsaturated or hydrogenated naturally occurring glyceride-type fats and oils of animal or vegetable nature, such as tallow, hog fat, rapeseed oil, etc. In general, these greases are prepared by the alkali fusion of the glyceride-type fat or oil in the presence of the lubricating oil menstruum. The amount of alkali metal base, e.g., sodium hydroxide, employed will be in excess of the amount required for saponification of the glycerides. The temperatures employed during alkali fusion will generally be within the range of about 450° to 600° F., preferably about 480° to 570° F.

While the reaction mechanism is not fully understood, it is postulated that the alkali fusion of the glyceride-type

fats and oils results in the formation of an alkali metal soap and an alkali metal salt of low molecular weight carboxylic acid. Thus, the grease thickener in these greases is believed to be an alkali metal soap-salt complex. For the purposes of the invention, the sodium soap-salt complex thickened greases are preferred. In U.S. Patent No. 2,265,791, the preparation of such a grease from rapeseed oil as the saponifiable material is described.

More specifically, sodium soap-salt complex thickened greases may be prepared by slowly heating rapeseed oil with an excess of alkali in a lubricating oil to a temperature of about 350° to 380° F. to effect saponification. The amount of alkali used is about 75 to 125% in excess, preferably about twice that required to saponify the rapeseed oil. The temperature of the reaction mixture is then raised to at least about 425° F. at which temperature hydrogen gas evolution commences. The mixture is then heated to and maintained at a temperature of about 450° to 500° F. for about 1 to 4 hours, preferably for about 2 hours. It is believed that during this heating step the rapeseed oil soap breaks down to some extent to liberate glycerin. The glycerin in turn breaks down to produce acrolein, which is converted into the alkali metal salt of a low molecular weight acid by alkali fusion. Thus, the final product comprises a mixture of C<sub>18</sub> to C<sub>22</sub> fatty acid soaps with sodium acrylate in minor proportions, up to about 1 mol of sodium acrylate per mol of sodium soap of high molecular weight acids. Some sodium formate, sodium acetate, sodium propionate and the like may also be present.

In general, the sodium base greases will comprise about 3 to 50 wt. percent, preferably about 5 to 35 wt. percent, of the thickening agent, i.e. the sodium soap or the sodium soap-salt complex obtained by alkali fusion, and about 50 to 97 wt. percent, preferably about 65 to 95 wt. percent, of the lubricating oil. The greases may

5 The following example and tables are presented to illustrate the preparation and various characteristics of the improved sodium base greases of the invention.

#### EXAMPLE

A number of sodium base lubricating greases were irradiated by filling one ounce screw-top bottles to the neck with the lubricating grease, closing the bottle with a plastic screw-top to leave very little air in the container, and then lowering the bottles into the center of a cylindrical cobalt 60 source. The undisturbed radiation intensity of source used to irradiate greases A and B was about  $2.2 \times 10^6$  roentgens per hour, whereas an undisturbed radiation intensity of about  $1.74 \times 10^6$  roentgens per hour was used in the irradiation of grease C. All of the greases were irradiated for 168 hours at a temperature of about 100° F.

10 The greases had the following formulations:

| Grease A (prepared by alkali fusion):      | Wt. percent |
|--------------------------------------------|-------------|
| Rapeseed oil                               | 22.0        |
| Sodium hydroxide                           | 4.75        |
| Sodium petroleum sulfonate                 | 1.00        |
| Di-salicylal propylene diamine             | 0.50        |
| Phenyl alpha-naphthylamine                 | 1.00        |
| Mineral lubricating oil, 55 SUS at 210° F. | 70.75       |

#### Grease B:

|                                            |       |
|--------------------------------------------|-------|
| Hydrogenated fish oil acids (sap. No. 190) | 15.0  |
| Sodium hydroxide                           | 2.55  |
| Mineral lubricating oil—                   |       |
| 50 SUS at 210° F.                          | 38.70 |
| 181 SUS at 210° F.                         | 43.75 |

#### Grease C:

|                                            |      |
|--------------------------------------------|------|
| Sodium stearate                            | 12.0 |
| Mineral lubricating oil, 55 SUS at 210° F. | 88.0 |

30 The effect of gamma ray irradiation on the above greases is set forth in the following table:

Table

| Grease | Change in |           | Dropping Point ° F. |       |        | Micro Penetration, mm./10 |       |
|--------|-----------|-----------|---------------------|-------|--------|---------------------------|-------|
|        | Color     | Odor      | Before              | After | Change | Before                    | After |
| A      | Lighter   | Less Odor | 500+                | 500+  | 0      | 79                        | 78    |
| B      | (1)<br>do | (2)       | 386                 | 390   | +4     | 85                        | 88    |
| C      | Lighter   |           | 374                 | 410   | +36    | 203                       | 243   |

<sup>1</sup> No change noticeable since base oil is dark green-black.

<sup>2</sup> No change in odor since it was odorless to begin with.

also contain minor proportions of conventional grease additives. More particularly, they may contain oxidation inhibitors (e.g. phenyl alpha-naphthylamine and di-tertiary butyl para cresol), metal deactivators, rust inhibitors, dyes, etc.

55 The irradiation of the sodium base greases may be carried out by a variety of procedures. For example, the radioactive source may be placed in a tank containing the greases to carry out a batch operation or the radioactive source may be placed into a stream of the grease for a continuous or semicontinuous operation. Many obvious modifications of these procedures will be apparent to those skilled in the art. The utilization of radiation emitted by radioactive material will necessitate, of course, adequate radiation shielding means and techniques. Such means and techniques are, however, well known in the art and need not be described here in detail.

60 The irradiation of the sodium base greases may be generally carried out at temperatures within the range of about -20° to 400° F. or higher. In general, the irradiation will be carried out at a temperature of about 50° to 200° F., preferably about 78° to 130° F. and under vacuum or elevated pressures, such as about 2 to 50 atmospheres. However, one of the advantages of the present process is that it may be effectively utilized at room temperature and at atmospheric pressure.

The above data show that physical properties of sodium base lubricating greases can be improved by subjecting the greases to high intensity ionizing radiation comprising gamma rays. Greases A and C both showed color improvement after irradiation, while greases A and B showed odor improvement. In addition, both greases B and C had higher dropping points following gamma ray irradiation; grease A having already such a high dropping point that no improvements can be measured with conventional methods.

65 It will be further understood that the invention is not necessarily limited to the specific materials and operating conditions of the foregoing examples. These materials and conditions may be varied within the limits indicated in the general portions of the specification.

What is claimed is:

1. A method of improving the dropping point of a lubricating grease consisting essentially of a major proportion of a mineral lubricating oil and a thickening amount of a sodium soap of a carboxylic acid having 12 to 30 carbon atoms per molecule, which comprises exposing said grease to an amount of gamma radiation sufficient to increase the dropping point of said grease and 70 within the range of  $10^5$  to  $3 \times 10^{10}$  roentgens, and recover-

ing a lubricating grease having an increased dropping point.

2. The method of claim 1 wherein said sodium soap is sodium stearate.

3. The method of claim 1 wherein the amount of said gamma radiation is within the range of  $10^6$  to  $3 \times 10^9$  roentgens.

References Cited in the file of this patent

UNITED STATES PATENTS

|           |                       |                |
|-----------|-----------------------|----------------|
| 2,637,695 | McKinley et al. ----- | May 5, 1953    |
| 2,719,122 | Morway -----          | Sept. 27, 1955 |
| 2,743,223 | McClinton -----       | Apr. 24, 1956  |

FOREIGN PATENTS

|         |                     |               |
|---------|---------------------|---------------|
| 154,213 | Great Britain ----- | Apr. 24, 1922 |
| 665,263 | Great Britain ----- | Jan. 23, 1952 |
| 66,034  | France -----        | Dec. 12, 1955 |

(4th addition of No. 1,079,401)

OTHER REFERENCES

Mincher: KAPL-731, pp. 3-8, Apr. 2, 1952. Declassified Feb. 15, 1955.

10 "Chem. and Eng. News," vol. 35, No. 17, page 28, April 29, 1957.

"Proceedings of the Second United Nations International Conference on the Peaceful Uses of Atomic Energy," vol. 29, pp. 276-286 (1958).